

## UNITED STATES PATENT OFFICE

2,150,400

## LUBRICATING OIL COMPOSITION

Raphael Rosen, Cranford, N. J., assignor to Standard Oil Development Company, a corporation of Delaware

No Drawing. Application October 4, 1934.  
Serial No. 746,844

## 6 Claims. (Cl. 87—9)

The present invention relates to improved lubricating oils and to methods for producing the same, and more specifically to a new class of oxidation inhibitors and to the oils of low oxidation rate containing such inhibitors. The invention will be fully understood from the following description:

It has been known for some time that hydrocarbon and other lubricating oils deteriorate by oxidation, and especially the more highly refined oils, particularly hydrocarbon oils which consist essentially of paraffin hydrocarbons. Such deterioration by oxidation may be controlled by the addition of substances known as oxidation inhibitors, of which the best known are phenols or naphthols and naphthyl amines, although a great many others are known.

The present application deals with a new class of oxidation inhibitors particularly useful for lubricating oils, including hydrocarbon lubricating oils, and these may be generally described as those containing an iso-cyanic radical which is represented by the formula —XCN, where X represents either an oxygen or a sulphur atom. It is preferred to use esters of iso-cyanic and iso-thio-cyanic acids. The alkyl esters may be used, for example those of the lower alcohols, such as methyl, ethyl, the propyl and butyl alkyl esters, either straight chain or with branch chain structures, such as isopropyl and secondary butyl iso-cyanates. Higher alkyl esters may also be used as well as the esters of unsaturated alcohols such as allyl iso-cyanate, vinyl iso-thio-cyanate and the corresponding propargyl esters, and the like. Di- and polyhydric alkyl esters of these acids may be used and these may be fully esterified or, if desired, only one of the two or more hydroxy groups need be esterified.

Besides the alkyl iso-cyanates and iso-thio-cyanates aryl esters may also be employed, such as the phenyl or naphthyl esters of the acids specified above, and of particular interest are the alkylated phenolic and naphtholic esters of such acids, which are more soluble in the oils than the corresponding unalkylated esters.

The esters may be added in relatively small amounts; for example as little as .1% is effective, although more is generally used, say from .2% to .5%. On the other hand, as much as 1% is generally unnecessary. These compounds may be added to the oil as such and dissolved in some solvent such as benzol or toluol and dispersed through the heavier oil.

The oils in which the present class of inhibitors may be used are generally described as well

refined lubricating oils. Petroleum lubricating oils may be obtained from any desirable crude source, such as paraffin, asphalt or mixed base crudes, and may be refined by ordinary methods, such as distillation, acid and clay treatment, or by special methods including hydrogenation, destructive hydrogenation, solvent extraction and heavy acid treatment with concentrated or fuming acid or oleum such as is used for the preparation of "white" oils for medicinal or technical purposes.

While cyanides and cyanates and cyanuric acid compounds have been used for various purposes in conjunction with hydrocarbon and other oils, it will be understood that the iso-cyanates and the iso-thio-cyanates are a quite different class of compounds and in general are much more effective for the present purposes than the cyanocompounds known hitherto. As examples of the action of the present class of compounds, the following may be considered:

## Example 1

To a petroleum lubricating oil, S. A. E. 50 grade, is added .2% of allyl iso-thio-cyanate, and this sample along with a blank sample of the oil containing none of the inhibitor were subjected to an oxidation test. A third sample containing ethyl thio-cyanate was subjected to test. The test was conducted by passing a stream of oxygen through a 10 cc. sample of oil which was held at 200° C. The gas stream was confined to a circulatory path and at fifteen-minute intervals the volume of oxygen absorbed was measured by difference. The result of these tests is included in the following table:

| Oil sample                                 | Oxygen absorption<br>cc. of oxygen/10<br>cc. sample/15-<br>minute intervals<br>at 200° C. |
|--------------------------------------------|-------------------------------------------------------------------------------------------|
| Lubricating oil (blank)                    | 190—80—63                                                                                 |
| Same containing .2% allyl iso-thio-cyanate | 18—100                                                                                    |
| Same containing .2% ethyl-thio-cyanate     | 171—94                                                                                    |

The above quoted results indicate that the thio-cyanate produced little, if any, reduction in oxidation rate while the iso-thio-cyanate greatly reduced the rate.

## Example 2

Samples of the oils used above were then subjected to a cone deposit test, which measures the tendency of oils to deposit sludge at elevated

temperatures. In these tests the oil was passed at a fixed rate through a groove cut in the inner surface of a steel cone of standardized dimensions which is heated to 250° C. After a fixed volume of the oil has passed through the cone the naphtha insoluble residue adhering to the cone and contained in the oil is collected and recorded. In these tests the blank sample showed a value of .42 gs. per 60 cc. of the oil against .29 for the sample containing the inhibitor.

*Example 3*

Another sample of a mineral lubricating oil S. A. E. 50 grade was subjected to the oxidation test along with two samples containing .2% of phenyl iso-cyanate and phenyl iso-thio-cyanate, respectively. The oxidation rates obtained are included in the following table:

| 20    | Sample                         | Oxygen absorption<br>cc. of oxygen/10<br>cc. sample/15-<br>minute interval |
|-------|--------------------------------|----------------------------------------------------------------------------|
| Blank |                                | 180-90-86                                                                  |
| 25    | Same + .2% phenyl iso-cyanate  | 70-95-70                                                                   |
|       | Same + phenyl iso-thio-cyanate | 16-68-120                                                                  |

The lubricating oils described above may contain additional ingredients, such as dyes for cast

or color, thickeners, pour inhibitors, soaps, dispersing agents and the like.

The invention is not to be limited to any theory of the action of the oxidation inhibitors nor to any particular oil nor to any particular inhibitor, but only to the following claims in which it is desired to claim all novelty inherent in the invention.

I claim:

1. Composition of matter comprising a viscous mineral lubricating oil and a small amount of an iso-cyanic compound selected from the class consisting of acids and esters soluble therein.
2. Composition of matter comprising a viscous mineral lubricating oil and a small amount of an ester selected from the class of alkyl and aryl esters of iso-cyanic acids.
3. Composition according to claim 2 in which the ester is an ester of iso-cyanic acid.
4. Composition according to claim 2 in which the ester is an ester of iso-thio-cyanic acid.
5. Composition according to claim 2 in which the added substance is an alkyl ester of an iso-cyanic acid.
6. Composition according to claim 2 in which the added substance is an alkyl ester of iso-thio-cyanic acid.

20  
25  
RAPHAEL ROSEN.

## DISCLAIMER

2,150,400.—*Raphael Rosen*, Cranford, N. J. LUBRICATING OIL COMPOSITION. Patent dated March 14, 1939. Disclaimer filed June 10, 1940, by the assignee, *Standard Oil Development Company*.

Hereby enters this disclaimer to claim 4 of said Letters Patent.  
[Official Gazette July 2, 1940.]